

## UNITED STATES PATENT OFFICE

JOHN C. BLACK AND WIRT D. RIAL, OF LOS ANGELES, CALIFORNIA, ASSIGNEES, BY  
MESNE ASSIGNMENTS, TO RICHFIELD OIL COMPANY OF CALIFORNIA, OF LOS  
ANGELES, CALIFORNIA, A CORPORATION OF DELAWARE

## PROCESS OF REFINING LUBRICATING OILS

No Drawing.

Application filed April 27, 1927. Serial No. 187,110.

This invention relates to an improved process for refining petroleum oils for the manufacture of lubricating oils.

This process is particularly adaptable for refining lubricating oil stocks derived from California petroleum, or other oils of like chemical composition, containing a high percentage of hydrocarbons of the carbocyclic series. Lubricating oil stocks derived from California crude petroleum oils, or other crude asphalt base petroleum oils, contain certain small percentages of organic acids, sulphur compounds, and unstable unsaturated hydrocarbon oils which must be removed before a stable lubricating oil can be produced.

By well known methods asphalt base lubricating oil stocks derived by distillation of an asphalt, or mixed base crude petroleum oil, of the required viscosity are treated with sulphuric acid and caustic soda, in quantities sufficient to remove the major part of said undesirable constituents, but there are still left in the lubricating oil stocks certain small percentages of undesirable constituents, produced by a polymerization and oxidation action during the said sulphuric acid treatment which remain dissolved in the finished lubricating oil and cannot be completely removed from all the stock by any known method; whereby the said finished lubricating oil will not conform to specifications as required by the United States Government for turbines, dynamos, and high speed steam engines, these oils being known as class "B" oils, which are outlined in the United States Government specifications, Bureau of Mines Technical Paper 323-A, page 11, test #9. The test required for this class of oils states that class "B" oils shall not form a permanent emulsion when agitated with a normal caustic soda solution.

We have determined that the compounds which cause a lubricating oil stock to emulsify with a solution of caustic soda are polymerized products, oxidized products, and oil soluble sulfo-compounds.

We are aware that a small percentage of a non-emulsifiable turbine oil stock may be made from a California or asphalt base lu-

bricating oil by a percolation filtration of the same through Florida fuller's earth, in which ten to twenty percent of the first oil coming through the filter will have non-emulsifying properties to a normal caustic soda solution, but the balance of the stock eighty to ninety percent will not meet said United States Government specifications required for class "B" oils.

These heretofore stated impurities present in California or asphalt base lubricating oil stocks, made by well known methods, not only render to the oil emulsifying properties, but also render such oil stocks unstable in color, whereby asphalt base lubricating oil stocks made by these well known methods may when stored for a period of time turn a darker color and acquire an undesirable blue bloom or fluorescence, which we believe is due to a continuation of polymerization promoted by said impurities in the oil.

We have discovered that these difficulties can be overcome and a lubricating oil stock produced which will retain its original color.

Our invention consists in the removal of a part of the above mentioned impurities before the acid treating operation and before any substantial oxidation can take place, while the lubricating oil stocks are being distilled, by introducing and commingling immediately therewith a water solution of caustic potash at a pressure and temperature sufficient to combine with said impurities, in quantities sufficient to extract therefrom substantially all the oxygen bearing hydrocarbons such as organic acids, aldehydes, and certain sulphur bearing hydrocarbons such as, hydrogen sulphide, and other unstable sulphur bearing compounds unknown in name and chemical composition to the inventors, separating the caustic potash containing the dissolved impurities from the lubricating oil distillate, treating said lubricating oil distillate with sulphuric acid in quantities sufficient to combine substantially with all the unstable hydrocarbons, and unstable sulphur bearing hydrocarbons with the formation of sulfo-acids or sludge, separating the acid treated oil from the sulfo-acids or sludge formed by said acid

treatment, then treating said separated oil with a comminuted solid adsorbent agent at temperatures suitable to decompose and adsorb all the soluble and suspended sulfo-acids remaining in said acid treated oil, and producing thereby an oil substantially free of mineral acid, then distilling therefrom the lighter grades of lubricating oil under vacuum to separate said lighter grades of lubricating oil from the heavier grades or cylinder stocks, and finally clarifying, purifying and decolorizing to the desired degree according to pending application of John C. Black et al., Serial Number 104,836, filed April 26, 1926.

The following describes the preferred method for carrying out our invention.

Lubricating oil distillate derived from the vacuum distillation, by any preferred method, of a California, Mexican, Texas, or other asphalt base crude petroleum oil, as it comes from the condenser and after passing through the "look-box", is continuously commingled with approximately 5% by volume of a 10° Beaumé caustic potash solution, by passing the same through a chamber filled with baffle plates, and then into a tank or agitator provided with an open steam pipe extending to or near the bottom of said agitator, by means of which said caustic potash solution and lubricating oil distillate are agitated with open steam and at a pressure of approximately 50 pounds gauge, until the temperature is raised to approximately 280° F. The mixture of oil and caustic potash solution is then permitted to rest in quiet without releasing the pressure until the caustic potash containing the dissolved impurities settles to the bottom of said agitator and is drawn off.

The caustic potash treated oil is then washed with water until substantially free of alkali, cooled and then treated in another agitator with 66° Beaumé sulphuric acid at a rate of approximately 40 pounds of said acid per barrel of oil charged, after which most of the sulfo-acid or sludge formed by said acid treatment is separated from the treated oil. This acid treated oil is then rendered free of mineral acidity by the so called "hot contact neutralizing process", as outlined in United States Patent of James W. Weir, Number 1,564,501, which comprises treating a lubricating oil stock after treatment with sulphuric acid with a comminuted solid adsorbent, agitating and heating the mixture to a temperature ranging from 180 to 350 degrees F., and then separating the treated lubricating oil stock from the solid adsorbent and adsorbed constituents. The oil free of mineral acidity is then subjected to a second distillation under vacuum, whereby the higher grades of lubricating stocks desired are separated from

the heavier grades of lubricating oil, or cylinder stocks.

The said cylinder stocks remaining in the still may be finished for what is known as bright stock, according to the pending application of John C. Black et al., Serial Number 104,836, filed April 26, 1926, or by other methods known in the art. The redistilled oils or lighter grades of lubricating oil may be finished to meet the specifications of class "B" oils as outlined in the United States Government specifications, Bureau of Mines Technical Paper 323-A, page 11, test No. 9, by a final clarifying and decolorizing operation employing the process as outlined in pending application of John C. Black et al., Serial Number 104,836, filed April 26, 1926, which comprises commingling the redistilled lubricating oil stock with a mixture of an adsorbent clay and an alkaline earth metal compound, such as calcium hydroxide at a temperature of approximately 300 degrees F., and separating the purified oil from the alkaline earth metal compound and adsorbent clay containing the emulsifiable constituents.

While the process herein described is well adapted for carrying out the objects of the present invention, it is understood that various modifications may be made without departing from the invention and the invention includes all such modifications and changes as come within the scope of the appended claims.

We claim:

1. That step in the method of treating lubricating oil stocks which consists in treating the same with a water solution of caustic potash agitating with steam under a pressure greater than atmospheric, and at a temperature of approximately 280 degrees F., in quantities sufficient to combine with the emulsifying constituents to be separated, dissolving the combined emulsifying constituents of the same therein, and separating the two liquids.

2. That step in the method of treating lubricating oil stocks derived from an asphalt base crude petroleum oil, which consists in treating the same with a water solution of caustic potash agitating with steam under pressure greater than atmospheric, and at a temperature of approximately 280 degrees F., in quantities sufficient to combine with the emulsifying constituents to be separated, dissolving the combined emulsifying constituents of the same therein, and separating the two liquids.

3. A method of treating lubricating oil stocks, which consists in treating the same with a water solution of caustic potash under pressure greater than atmospheric, and at a temperature of approximately 280 degrees F., in quantities sufficient to combine with the emulsifying constituents to be separated, dis-

solving the combined emulsifying constituents of the same therein, and separating the two liquids, then treating said separated lubricating oil stocks with sulphuric acid in quantities sufficient to combine with all the unstable hydrocarbons contained therein, separating the acid treated lubricating oil stocks from the unstable hydrocarbons combined with said sulphuric acid, then treating said acid treated lubricating oil stocks with a solid adsorbent material at temperatures greater than 200° F., in quantities sufficient to decompose and adsorb all the sulfo-acid constituents contained therein which were produced and not separated by said acid treatment, separating said solid adsorbent material containing the adsorbed sulfo-acid constituents from the treated lubricating oil stocks, separating the lighter grades of lubricating oil stocks from the heavier grade of lubricating oil stock by a vacuum distillation, and finally clarifying and decolorizing to the desired degree.

4. A method of treating lubricating oil stocks derived from an asphalt base crude petroleum oil, which consists in treating the same with a water solution of caustic potash under a pressure greater than atmospheric, and at a temperature of approximately 280 degrees F., in quantities sufficient to combine with the emulsifying constituents to be separated, dissolving the combined emulsifying constituents of the same therein, and separating the two liquids, then treating said separated lubricating oil stocks with sulphuric acid in quantities sufficient to combine with all the unstable hydrocarbons contained therein, separating the acid treated lubricating oil stocks from the unstable hydrocarbons combined with said sulphuric acid, then treating said acid treated lubricating oil stocks with a solid adsorbent material at temperatures greater than 200° F., in quantities sufficient to adsorb all the sulfo-acid constituents containing therein which were produced and not separated by said acid treatment, separating said solid adsorbent material containing the adsorbed sulfo-acid constituents from the treated lubricating oil stocks, separating the lighter grade of lubricants from the heavier grade of lubricating oil stock by vacuum distillation after said treatment with a solid adsorbent material, and finally clarifying and decolorizing to the desired degree.

5. A method of producing a lubricating oil which will not emulsify when commingled with a water solution of caustic soda, which consists in treating a lubricating oil distillate with a water solution of caustic potash, under a pressure greater than atmospheric and at a temperature of approximately 280 degrees F., in quantities sufficient to combine with the emulsifying constituents to be separated, dissolving the combined emulsifying

constituents of the same therein, and separating the two liquids, then treating said separated lubricating oil stocks with sulphuric acid in quantities sufficient to combine with substantially all the unstable hydrocarbons contained therein, separating the acid treated lubricating oil stocks from the unstable hydrocarbons combined with said sulphuric acid, then treating said acid treated lubricating oil stocks with a solid adsorbent material at temperatures greater than 200° F., in quantities sufficient to adsorb all the sulfo-acid constituents contained therein, which were produced and not separated by said acid treatment, separating said solid adsorbent material containing the adsorbed sulfo-acid constituents from the treated lubricating oil stocks, separating the lighter grade of lubricating oil stock from the heavier grade of lubricating oil stock, by a vacuum distillation, and finally clarifying and decolorizing to the required degree, with a decolorizing agent mixed with an alkaline metal hydroxide.

6. The step in the method of improving the color and demulsifying qualities of lubricating oils which comprises heating the lubricating oils at a temperature of approximately 280 degrees F. with a caustic potash solution under pressure prior to acid treatment thereof.

7. The step in the method of improving the color and demulsifying qualities of lubricating oils which comprises heating the lubricating oils at a temperature of approximately 280 degrees F. with a caustic potash solution under pressure prior to acid treatment thereof, allowing the mixture to stratify and washing the oil layer to free it from alkali.

In testimony whereof we affix our signatures.

JOHN C. BLACK,  
WIRT D. RIAL.

110

115

120

125

130